

# United States Patent Office

2,775,516

Patented Dec. 25, 1956

1

2,775,516

## METHOD FOR PRODUCTION OF COMPOUND IRON POWDERS

William M. Shafer, Johnstown, Pa., assignor to The National-U. S. Radiator Company, a corporation of Maryland

No Drawing. Application June 17, 1954,  
Serial No. 437,569

7 Claims. (Cl. 75—5)

In the production of iron articles by powder metallurgy a common practice is to add to the iron powder various non-ferrous metals for the development of certain properties, for instance to improve the strength or the corrosion resistance of pressed and sintered parts. Certain difficulties and disadvantages attend that practice. For instance, there is always the problem of obtaining the necessary intimate mixture of the two metal powders and of maintaining its homogeneity during handling and in the pressing operations. Especially disadvantageous is the effect produced by some non-ferrous metal powders, notably copper, of causing an undesirable growth of parts sintered from mixtures of them with most iron powders. Such increase in dimensions is objectionable in that it makes it difficult to produce accurately sized parts.

It is among the objects of this invention to provide iron powders compounded with non-ferrous metals that are easily and inexpensively produced; that avoid the foregoing disadvantages of the previous practice of mixing powders of iron and non-ferrous metals; that produce stronger pressed and sintered parts than are to be obtained by the previous practices; that undergo little or no positive growth during sintering; and which may be pressed and sintered without modification of existing practices in those operations.

Other objects will appear from the following specification:

The invention is predicated upon my discovery that the troubles and disadvantages encountered in the existing practice of mixing iron powder with a non-ferrous metal powder are obviated by a compound iron powder produced by heating a mixture of (1) iron powder containing a substantial proportion of combined carbon and (2) finely divided oxide of a metal that is reducible by carbon. In the practice of the invention the iron powder and oxide are mixed intimately and heated in a closed container or in a non-oxidizing atmosphere. Decarburization of the iron occurs with concurrent reduction of the non-ferrous metal oxide to metal which becomes deposited on the surface of the iron powder particles. This powder may then be used in accordance with standard practices for the pressing and sintering of parts without the occurrence of stratification of the non-ferrous metal or development of non-homogeneity, thus avoiding the segregation that tends to occur when simple mixtures of the two powders are used.

A major advantage of the compound powder made in accordance with this invention is that the growth, or increase in dimensions, that occurs with mixtures of most iron powders with copper is avoided, with, usually, an actual decrease in dimensions such as is desirable. Attendant also upon the use of these new compound iron powders is the advantageous fact that sintered strength is greater than with simple mechanical mixtures of the same composition.

The composition of the mixture of iron powder containing combined carbon and non-ferrous metal oxide will depend upon the content of non-ferrous metal desired in the compound powder, and also upon the content of combined carbon in the original iron powder and the

2

amount of carbon desired in the final product. For many purposes the two are mixed in proportions such that the iron powder will be decarburized, or at least have its carbon content reduced to a low value, say not more than about 0.2 percent, while effecting reduction of all of the non-ferrous metal oxide. However, for some purposes, as where steel parts susceptible to hardening by heat treatment are desired, the residual carbon in the compound powder may be as desired. In such instances, and especially where relatively large amounts of non-ferrous metal are to appear in the compound powder, it is desirable that the starting iron powder contain a high proportion of carbon as iron carbide. If only small amounts of non-ferrous metal oxide are to be reduced, desirably the combined carbon content of the iron powder will be only such as to reduce the oxide leaving the iron powder decarburized or substantially so.

In instances when it is desired to keep the non-ferrous metal content lower than it could be kept if enough non-ferrous metal oxide were added to sufficiently decarburize the iron, sufficient decarburization is achieved by including an appropriate amount of iron oxide in the mixture. Mill scale suffices for this purpose but other iron oxides may be used.

25 Inasmuch as copper is the non-ferrous metal most commonly used with iron powder, the invention may be described in further detail with reference to a compound iron-copper powder. The carbon-containing iron powder is mixed with the appropriate amount of finely divided cuprous or cupric oxide in proportions that are approximately stoichiometric with respect to the total amount of carbon present and the amount of oxide to be reduced. The iron powder and oxide are intimately mixed and then heated at 1600° to 1900° F. in a closed container or in a furnace provided with a non-oxidizing atmosphere that is inert to iron and the metal of the oxide. As exemplifying the benefits to be derived from the invention, reference may be made to the following tests:

*Powder A.*—100-mesh ground high carbon iron shot was decarburized with 100-mesh mill scale at 1650° F. in a protective atmosphere and then mixed with 11 percent by weight of 100-mesh pure copper powder.

*Powder B.*—Twenty pounds of 100-mesh high carbon ground shot containing 3.07 percent of carbon and 2.82 percent of oxygen were mixed with 3.28 pounds of copper oxide and 2.37 pounds of 100-mesh mill scale. The mixture was heated as with Powder A.

*Powder C.*—A mixture of, by weight, 77.7 percent of ground 100-mesh iron shot containing 2.88 percent total carbon and 1.46 percent of oxygen, 10 percent of 100-mesh mill scale, and 12.3 percent of 100-mesh copper oxide was heated like Powders A and B.

55 Standard tensile bars were pressed at 30 tons per square inch using one percent of added zinc stearate as a lubricant, and the bars were sintered in hydrogen for thirty minutes at 2020° F. The composition of Powders A to C and the properties of the tensile bars thus produced were as follows:

| 60 | Powder No. | Powder Composition                                                            | Growth, Percent |        | Ult. T. S., p.s.i. | Elong., Percent |
|----|------------|-------------------------------------------------------------------------------|-----------------|--------|--------------------|-----------------|
|    |            |                                                                               | Axial           | Radial |                    |                 |
| 65 | A-----     | Iron plus 11% added Cu. Total C—0.14%; O <sub>2</sub> —0.6%.                  | +1.03           | +1.04  | 30,700             | 1.0             |
|    | B-----     | Iron plus 11% Cu by oxide reduction. Total C—0.12%; O <sub>2</sub> —0.6%.     | -0.80           | -0.44  | 40,050             | 1.0             |
| 70 | C-----     | Iron plus 10.65% Cu by oxide reduction. Total C—0.11%; O <sub>2</sub> —0.27%. | -0.04           | +0.61  | 48,000             | 1.0             |

It will be observed that there was substantial growth, both axially and radially in the case of the simple mechanical mixture of iron and copper powder. In marked contrast, in the case of Powders B and C produced in accordance with this invention there was actual slight shrinkage in both directions with Powder B, axial shrinkage in the case of Powder C and only slight growth radially. The data show also the very substantial increase in strength of the bars pressed from Powders B and C as compared with those made from Powder A.

Although the invention has been described with particular reference to compound iron-copper powder, it is applicable also to other non-ferrous oxides, as evidenced by the following series of tests:

*Powder D.*—100-mesh annealed iron powder was mixed with 6 percent by weight of 325-mesh pure nickel powder.

*Powder E.*—A mixture of, by weight, 81.28 percent of the ground high carbon shot used in producing Powder C, 9.36 percent of nickel oxide, and 9.36 percent of 100-mesh mill scale was heated at 1650° F. in a protective atmosphere.

*Powder F.*—100-mesh annealed iron powder was mixed with one percent by weight of 325-mesh pure nickel powder.

*Powder G.*—A mixture of, by weight, 81.3 percent of the iron powder used in making Powder C, 17.4 percent of 100-mesh mill scale, and 1.3 percent of nickel oxide was heated in the same manner used in producing Powder E.

Powders D to G were used for the production of tensile bars in the same manner as was done with Powders A to C. The composition of these powders and the test data are shown in the following table:

| Powder No. | Powder Composition                                                           | Growth, Percent |        | Ult. T. S., p. s. i. | Elong., Percent |
|------------|------------------------------------------------------------------------------|-----------------|--------|----------------------|-----------------|
|            |                                                                              | Axial           | Radial |                      |                 |
| D-----     | Iron plus 6% added Ni.                                                       | -1.19           | -0.578 | 8,750                | 2.0             |
| E-----     | Iron plus 7.22% Ni by oxide reduction. Total C—0.10%; O <sub>2</sub> —0.32%. | -1.55           | -0.96  | 22,650               | 2.0             |
| F-----     | Iron +1.0% added Ni.                                                         | -0.865          | -0.378 | 13,900               | 5.0             |
| G-----     | Iron plus 1.08% Ni by oxide reduction. Total C—0.22%; O <sub>2</sub> —0.59%. | -0.69           | -0.64  | 15,180               | 2.8             |

These data again show the shrinkage that characterizes the compound powders of this invention coupled with increase in strength as compared with articles made in the same way from mere mechanical mixtures of the same or closely similar composition.

Other oxides of non-ferrous metals may be used, if desired, for the development of special properties, examples being oxides of cadmium, lead, tin, bismuth, molybdenum and cobalt. Also, two or more such oxides may be present in the mixtures to be reduced.

According to the provisions of the patent statutes, I have explained the principle of my invention and have described what I now consider to represent its best embodiment. However, I desire to have it understood that, 10 within the scope of the appended claims, the invention may be practiced otherwise than as specifically described.

I claim:

1. That method of making compound iron powder comprising mixing iron powder containing combined carbon with at least one finely divided oxide of a non-ferrous metal reducible by carbon, heating the mixture under non-oxidizing conditions to a temperature at which said oxide is reduced by the carbon of said powder, and recovering iron particles of lowered carbon content surface coated with the metal of said oxide.
2. A method according to claim 1, said oxide being selected from the group consisting of oxides of copper and nickel.
3. A method according to claim 2, said mixture also containing an iron oxide.
4. That method of making compound iron powder comprising mixing iron powder containing combined carbon with at least one finely divided oxide of a non-ferrous metal reducible by carbon, the proportions of said powder and oxide being such as to provide carbon in an amount to reduce said oxide with production of iron powder of low carbon content, heating the mixture under non-oxidizing conditions to a temperature at which said oxide is reduced by the carbon of said powder, and recovering iron particles of lowered carbon content surface coated with the metal of said oxide.
5. A method according to claim 4, said mixture containing also an iron oxide.
6. A method according to claim 5, said non-ferrous metal oxide being selected from the group consisting of oxides of copper and nickel.
7. A method according to claim 4, said oxide being selected from the group consisting of oxides of copper and nickel, and said heating being at 1600° to 1900° F.

References Cited in the file of this patent

UNITED STATES PATENTS

2,483,075 Truesdale ----- Sept. 27, 1949